

Nov. 21, 1972

KAIICHIRO SAKAZUME ET AL  
SUPERSENSITIZED LIGHT-SENSITIVE SILVER HALIDE  
PHOTOGRAPHIC EMULSION

Filed Dec. 23, 1970

3,703,377

Fig.1



Fig.2



Fig.3



Kaiichiro Sakazume, Eiichi Sakamoto, Shigemasa Itoh, Noboru Fujimori, Shigeji Baba INVENTORS

BY

Bierman & Bierman,

ATTORNEYS.

# United States Patent Office

3,703,377  
Patented Nov. 21, 1972

1

3,703,377

## SUPERSENSITIZED LIGHT-SENSITIVE SILVER HALIDE PHOTOGRAPHIC EMULSION

Kaijiro Sakazume, Tokyo, Eiichi Sakamoto, Hanno, Shigemasa Itoh and Noboru Fujimori, Tokyo, and Shigeji Baba, Zam-machi, Japan, assignors to Konishiroku Photo Industry Co., Ltd., Tokyo, Japan

Filed Dec. 23, 1970, Ser. No. 101,066

Claims priority, application Japan, Jan. 16, 1970,  
45/3,820

U.S. Cl. 96—122

Int. Cl. G03c 1/08

5 Claims

### ABSTRACT OF THE DISCLOSURE

The emulsion contains at least one compound of the formula



wherein P is



R<sub>2</sub> and R<sub>3</sub> are individually an alkyl group; X is S, O, N, or N—R wherein R is hydrogen, an alkyl group or a lower alkyl group; and R<sub>1</sub> is an alkyl, allyl or aryl group, in combination with at least one compound of the formula



wherein R<sub>4</sub> is an alkyl group; R<sub>5</sub> and R<sub>6</sub> are individually an alkyl or aryl group; and Z<sub>1</sub> and Z<sub>2</sub> are individually a hydrogen or halogen atom or an alkyl, alkoxy or aryl group, said Z<sub>1</sub> and Z<sub>2</sub> may link to each other to form a benzene ring. The emulsion when subjected to supersensitization displays ideal color sensitivity.

This invention relates to a light-sensitive silver halide photographic material containing a combination of sensitizing dyes, particularly to a so-called lith-type light-sensitive photographic material which gives a hard tone and a sharp dot image. More particularly, the invention pertains to a light-sensitive silver halide photographic emulsion characterized by containing at least one compound of the general formula



(I)

wherein P is



2

where R<sub>2</sub> and R<sub>3</sub> are individually an alkyl group; Q is a non-metallic atomic group necessary for forming a 5-membered ring; and R<sub>1</sub> is an alkyl, allyl or aryl group, in combination with at least one compound of the general formula



wherein R<sub>4</sub> is an alkyl group; R<sub>5</sub> and R<sub>6</sub> are individually an alkyl or aryl group; and Z<sub>1</sub> and Z<sub>2</sub> are individually a hydrogen or halogen atom or an alkyl, alkoxy or aryl group, said Z<sub>1</sub> and Z<sub>2</sub> may link each other to form a benzene ring.

As is well known, the inherent light-sensitive wavelength region of a silver halide emulsion is ordinarily an extremely limited short wavelength region (400 m $\mu$  or less) of ultraviolet ray or blue light. It is well known that as a means for the spectral sensitization of such silver halide emulsion, the use of certain cyanine dye is markedly effective. It is also well known that when a combination of the above-mentioned sensitizing dye and a certain other sensitizing dye or an organic compound is added to a silver halide emulsion, light sensitivity greater than that recognized as the sum of the sensitizing effects of the individual compounds can be imparted to the emulsion. Such effect is called as supersensitization, and many combinations of compounds have already been reported.

In applying such supersensitization method to a silver halide emulsion, particularly a lith-type silver chlorobromide emulsion, it is desirable that not only the increase in color sensitization effect is attained but also such conditions as set forth below are satisfied.

(1) The supersensitization method does not disturb the characteristics of the lith-type emulsion which has an extremely high contrast.

(2) The supersensitization method should contribute to the improvement in fine dot quality of a half-tone image without deteriorating the sharpness thereof.

(3) The supersensitization method should not bring about any dye stain or fog on the film after high contrast development.

Further, it is desirable that in the case of a lith-type silver chlorobromide emulsion which requires a visible wavelength region, particularly a blue light- or green light-sensitive region, the supersensitization shows high sensitivity in the blue light-sensitive region without desensitizing the inherent sensitivity thereof and provides sharp and good dots by development within such a relatively short period of time as 2 to 3 minutes.

However, most of the conventional supersensitization methods and chiefly employed for the treatment of ordinary silver iodobromide emulsions for negatives, and the actual state is such that neither of said methods can satisfy the aforesaid conditions when applied to high contrast silver chlorobromide emulsions.

An object of the present invention is to provide a light-sensitive silver halide photographic material which has been subjected to supersensitization capable of satisfying the aforesaid conditions.

Another object of the invention is to provide a light-sensitive silver halide photographic material which has no detrimental interactions with co-existing photographic additives and which maintains stabilized photographic properties even when stored for a long period of time.

As the result of extensive studies, we have found that when a combination of at least one compound of the General Formula I and at least one compound of the General Formula II is incorporated into a silver halide photographic emulsion, not only a marked increase in color sensitization effect can be attained but also all the aforesaid conditions can be satisfied.

Both of the compounds represented by the General Formulas I and II are merocyanine type sensitizing dyes, and when these sensitizing dyes are used in combination according to the present invention, spectral sensitivity maximum values exhibited by the individual sensitizing dyes can be brought to a unified collective maximum value to make it possible to attain the best ortho-sensitivity. That is due to synergistic effect derived from the specific combination of said compounds, the purple light region and green light region of emulsion are markedly enhanced in sensitization. Further, the combination of said compounds has such characteristic that when the compounds are added to a lith-type emulsion, to which is applied a lith developer containing hydroquinone as a principal ingredient together with aldehyde, it is possible to obtain a sharp dot image which is high in contrast.

Typical examples of the compounds of the General Formulas I and II are enumerated below, but compounds usable in the present invention are not limited only to these.

Typical examples of the compounds of the General Formula I are as follows:

(A)



Exemplified Compound No.

(1)  $-\text{CH}_3$   
(2)  $-\text{C}_2\text{H}_5$

(3)  $-\text{C}_2\text{H}_5$

(4)  $-\text{CH}_3$

(5)  $-\text{C}_2\text{H}_5$

(6)  $-\text{CH}_3$

(7)  $-\text{CH}_3$

(8)  $-(n)\text{C}_2\text{H}_5$

$-\text{CH}_2\text{CH}=\text{CH}_2$   
 $-\text{C}_2\text{H}_5$



(B)



Exemplified Compound No.

(9)  $-\text{CH}_3$

(10)  $-\text{C}_2\text{H}_5$

(11)  $-\text{CH}_3$

(12)  $-\text{CH}_3$

(13)  $-(\text{CH}_2)_3\text{S O}_3\text{K}$

(14)  $-\text{CH}_2\text{CH}_2\text{OH}$

(15)  $-\text{CH}_2-\text{CO}-\text{phenyl}$

(16)  $-\text{CH}_2\text{COO}-\text{C}_2\text{H}_5$

$-\text{C}_2\text{H}_5$



30

(C)



5

10

Exemplified Compound No.

(17)  $-\text{CH}_3$

(18)  $-\text{CH}_3$

(19)  $-\text{C}_2\text{H}_5$

(20)  $-\text{CH}_3$

(21)  $-\text{C}_2\text{H}_5$

$-\text{C}_2\text{H}_5$

$-\text{CH}_2\text{CH}_2\text{OH}$

$-\text{CH}_2\text{CH}_2\text{OCOCH}_3$

$-\text{CH}_2\text{CH}_2\text{SO}_3\text{K}$

15

$-\text{CH}_2\text{CH}_2\text{OH}$

$-\text{CH}_2\text{CH}_2\text{OCOCH}_3$

$-\text{CH}_2\text{CH}_2\text{SO}_3\text{K}$

20

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

4



5

10

15

20

25

30

35

40

45

5

Typical examples of the compounds of the General Formula II are as follows:

(31)



(32)



(33)



(34)



(88)



(78)



(37)

6



5



55 A light-sensitive photographic material, which has been subjected to supersensitization by incorporation of a specific combination of the above-mentioned compounds, has such excellent characteristics as mentioned previously, and can display ideal color sensitivity. Thus, the combination of said compounds imparts quite excellent properties not only to a lith-type light-sensitive material but also to a light-sensitive photographic material comprising other silver chloride or silver chlorobromide emulsion.

65 The distribution in sensitization maximum wavelength of a silver halide emulsion according to the present invention is variable depending on the kinds and proportions of the sensitizing dyes of the general Formulas I and II. The sensitizing dyes may be added in the form of a solution in a water-miscible organic solvent such as methanol or ethanol. Alternatively, each of the sensitizing dyes may 70 be added individually in the form of a solution in such organic solvent as mentioned above. The time of addition of said sensitizing dyes to a silver halide emulsion may be any stage during preparation of the emulsion, but is preferably after completion of the second ripening, in general. The amounts of the sensitizing dyes to be added 75

vary depending on the kind of the silver halide emulsion used. Ordinarily, however, the total amount of the sensitizing dyes of the General Formulas I and II is variable in a wide range of 1 mg. to 200 mg. per kg. of the silver halide emulsion. In this case, the mixing ratio of the sensitizing dye of the General Formula I to the sensitizing dye of the General Formula II is preferably 1:10 to 10:1 by weight.

Silver halide emulsions usable in the present invention include silver chloride, silver chlorobromide and silver bromide emulsions. These emulsions may have been incorporated with such sensitizers as noble metal and sulfur sensitizers, or with polyalkylene oxide type compounds as contrast-improving agents. Further, the emulsions may have been optically sensitized over the whole visible light regions by additional incorporation of other sensitizing dyes, e.g. carbocyanine dyes. Particularly when red light sensitivity is desired to be attained, the use of thiacyanocyanine dyes is preferable. The emulsions may further contain ordinary photographic additives such as stabilizers, hardeners, coating aids, etc.

The above-mentioned silver halide photographic emulsions containing the compounds are individually coated on a suitable support such as glass, cellulose triacetate base, polyester base or paper, and then dried, whereby the light-sensitive silver halide photographic materials of the present invention can be obtained.

The present invention is illustrated in further detail below with reference to examples, but the examples are illustrative and the invention is, of course, not limited to these.

#### EXAMPLE 1

A lith-type silver chlorobromide emulsion containing 2.0 mol percent of silver bromide which had been treated with a gelatin coagulant was subjected to second ripening according to gold sensitization method and then divided into several portions. Each divided emulsion was incorporated with methanol solutions of the exemplified compounds shown in Table 1, either singly or in combination of two. Subsequently, the emulsion was allowed to stand at about 40° C. for 20 minutes to stabilize sensitiveness, added with a suitable amount of a polyalkylene oxide derivative as a tone-hardening agent and further with a hardening agent and a coating aid, coated on a film base and then dried to prepare green-sensitive lith-type light-sensitive materials.

For comparison, a control sample was prepared in the same manner as above, except that the two sensitizing dyes (a) and (b) shown below which are disclosed in U.S. Pat. 2,977,229 were used in combination.

#### Control dyes



These samples were individually exposed to a light of 125 lux (2,660° K.) through blue and green filters having transmission maximums at 450 m $\mu$  and 525 m $\mu$ , respectively, using sensitometer Model KS-VII (manufactured by Konishiroku Photo Industry Co., Ltd.), and then developed at 20° C. for 3 minutes with a developer of the following composition:

|                                                     |     |     |
|-----------------------------------------------------|-----|-----|
| Hot water                                           | ml. | 500 |
| Addition product of formaldehyde and sodium sulfite | g.  | 50  |
| Hydroquinone                                        | g.  | 19  |
| Sodium carbonate                                    | g.  | 80  |
| Boric acid                                          | g.  | 10  |
| Potassium bromide                                   | g.  | 2.2 |
| Water to make 1,000 ml.                             |     |     |

The results obtained were as shown in Table 1. In the table, the relative speed is a value calculated by regarding as 100 the green light speed of the sample using the control dyes (a) and (b), and the dye stain is a density value measured by use of a complementary color filter.

TABLE 1

| Sample No. | Amounts of exemplified compounds added (mg./kg. emulsion) | Relative purple light speed | Relative green light speed | Residual color (dye stain) |
|------------|-----------------------------------------------------------|-----------------------------|----------------------------|----------------------------|
| 20         | Control dyes, (a) 30 mg. + (b) 30 mg.                     | 60                          | 100                        | 0.03                       |
| 2          | (1) 50 mg.                                                | 80                          | 60                         | 0.02                       |
| 3          | (34) 50 mg.                                               | 60                          | 90                         | 0.03                       |
| 4          | (1) 30 mg. + (34) 30 mg.                                  | 100                         | 150                        | 0.02                       |
| 5          | (9) 50 mg.                                                | 100                         | 50                         | 0.02                       |
| 6          | (35) 50 mg.                                               | 40                          | 80                         | 0.02                       |
| 7          | (9) 30 mg. + (35) 30 mg.                                  | 120                         | 170                        | 0.02                       |
| 8          | (19) 50 mg.                                               | 90                          | 60                         | 0.02                       |
| 9          | (37) 50 mg.                                               | 50                          | 85                         | 0.03                       |
| 10         | (19) 30 mg. + (37) 30 mg.                                 | 110                         | 140                        | 0.02                       |

As is clear from Table 1 and the drawings shown later, the samples incorporated with combinations of the compounds according to the present invention are more excellent in sensitization degree in individual sensitizing region than the samples incorporated with individual compounds, and are greater in speed and less in formation of dye stain than the control sample.

In the accompanying drawings, FIG. 1 shows a spectral sensitivity curve of a silver chlorobromide emulsion; FIG. 2 shows spectral sensitivity curves of the sample 2 (dotted line) and of the sample 3 (solid line); and FIG. 3 shows a spectral sensitivity curve of the sample 4 according to the present invention.

#### EXAMPLE 2

Example 1 was repeated, except that the divided emulsions were individually incorporated with each of such combinations of the exemplified compounds as shown in Table 2, to prepare green-sensitive lith-type light-sensitive photographic materials. The sensitometry of each sample was effected in the same manner as in Example 1 to calculate the relative speed thereof, and the contrast was expressed in terms of an average gradient between the point where the density was 0.5 and the point where the density was 2.0. The evaluation of dots was carried out in such a manner that the sample was brought into close contact with a contact screen exposed and then subjected to development under the same conditions as in the case of the sensitometry, and the resulting dots were visually investigated by means of a microscope. The evaluation of dots was represented by each of the ratings 1 to 5, assuming that the rating of dots which were free from fringes and highest in sharpness was 5, and the rating of dots which were extremely large in amount of fringes was 1. The control dyes used in this example were the same as in Example 1.

TABLE 2

| Sample No. | Amounts of exemplified compounds added (mg./kg. emulsion) | Relative purple light speed | Relative green light speed | Contrast | Evaluation of dots |
|------------|-----------------------------------------------------------|-----------------------------|----------------------------|----------|--------------------|
| 70         | Control dyes (a) 30 mg. + (b) 30 mg.                      | 60                          | 100                        | 8.0      | 2-3                |
| 12         | (4) 30 mg. + (32) 30 mg.                                  | 180                         | 230                        | 11       | 3                  |
| 13         | (4) 30 mg. + (35) 30 mg.                                  | 100                         | 150                        | 15       | 5                  |
| 14         | (11) 30 mg. + (38) 30 mg.                                 | 160                         | 220                        | 12       | 4                  |
| 15         | (11) 30 mg. + (34) 30 mg.                                 | 190                         | 200                        | 12       | 4                  |
| 16         | (22) 30 mg. + (39) 30 mg.                                 | 200                         | 240                        | 11       | 3                  |
| 17         | (22) 30 mg. + (41) 30 mg.                                 | 170                         | 190                        | 13       | 4                  |

As is clear from Table 2, the samples 12 to 17 according to the present invention showed markedly excellent characteristics as compared with the control sample in every respect of speed, contrast and dot quality.

## EXAMPLE 3

A silver chlorobromide emulsion containing 20 mol percent of silver bromide was subjected to second ripening and then divided into several portions, which were then individually incorporated with each of such combinations of exemplified compounds as shown in Table 3. Subsequently, the emulsions were sensitized in the red light region by addition of such amount as shown in Table 3 of a 1:1 mixture of anhydro-3,3'- $\gamma$ -sulfopropyl-9-ethyl-4,5,4',5'-dibenzothiacarbocyanine hydroxide (hereinafter referred to as "Red 1") and 3- $\gamma$ -sulfopropyl-9-ethyl-4,5-dibenz-3',8-sulfobutyl-5'-methylthiacarbocyanine sodium salt (hereinafter referred to as "Red 2"), and sufficiently stabilized in optical sensitization. Subsequently, the same additives as in Example 1 were added to prepare panchromatically sensitized lith-type light-sensitive materials.

The sensitometry of the thus prepared samples was carried out in such a manner that the samples were exposed to light through the blue and green filters used in Example 1 and a red filter capable of transmitting a light of more than 600  $\mu$  in wavelength, and then developed at 20° C. for 3 minutes with D-11 developer formulated by Eastman Kodak Co. The results obtained were as shown in Table 3. In the table, the relative speed is a value calculated by assuming as 100 the speed of a sample containing only the red-sensitive dye Red 1.

TABLE 3

| Sample No. | Amount of exemplified compounds added (mg./kg. emulsion)        | Relative purple light speed | Relative green light speed | Relative red light speed | Fog  |
|------------|-----------------------------------------------------------------|-----------------------------|----------------------------|--------------------------|------|
| 18.....    | Control sample containing only red-sensitive dye (Red 1) 20 mg. | 100                         | 100                        | 100                      | 0.08 |
| 19.....    | (5) 20 mg. + (33) 20 mg. + (Red 1) 20 mg. + (Red 2) 20 mg.      | 280                         | 190                        | 105                      | 0.08 |
| 20.....    | (14) 20 mg. + (31) 20 mg. + (Red 1) 20 mg. + (Red 2) 20 mg.     | 220                         | 160                        | 110                      | 0.09 |
| 21.....    | (26) 20 mg. + (38) 20 mg. + (Red 1) 20 mg. + (Red 2) 20 mg.     | 170                         | 130                        | 100                      | 0.08 |

From Table 3, it is understood that even when used together with a red-sensitive sensitizing dye, the samples incorporated with combination of the compounds according to the present invention have excellent photographic properties.

What we claim is:

1. A light-sensitive silver halide photographic emulsion characterized by containing at least one compound of the General Formula I,



(I)

wherein P is



R<sub>2</sub> and R<sub>3</sub> are individually an alkyl group; X is S, O, N or N—R where R is hydrogen, an aryl group or a lower

alkyl group; and R<sub>1</sub> is an alkyl, allyl or aryl group, in combination with at least one compound of the General Formula II,



15 wherein R<sub>4</sub> is an alkyl group; R<sub>5</sub> and R<sub>6</sub> are individually an alkyl or aryl group; and Z<sub>1</sub> and Z<sub>2</sub> are individually a hydrogen or halogen atom or an alkyl, alkoxy or aryl group, said Z<sub>1</sub> and Z<sub>2</sub> may link to each other to form a benzene ring.

20 2. The light-sensitive silver halide photographic emulsion as claimed in claim 1, wherein the compound of the General Formula I is one member selected from the group consisting of:



65

and



70

3. A light-sensitive silver halide photographic emulsion as claimed in claim 1, wherein the compound of the Gen-

11

11  
eral Formula II is one member selected from the group consisting of:



and



12

4. The light-sensitive silver halide photographic emulsion as claimed in claim 1, wherein the total amount of the compound of the General Formula I and that of the General Formula II is within the range of 1 mg. to 200 mg. per kilogram of said emulsion.

5. The light-sensitive silver halide photographic emulsion as claimed in claim 1, wherein said emulsion is of the lith-type.

10

### References Cited

UNITED STATES PATENTS

- 2,972,539 2/1961 Jones ----- 96-122  
2,977,229 3/1961 Jones ----- 96-126

15

## FOREIGN PATENTS

- 918.308 9/1954 Germany ----- 96-122

J. TRAVIS BROWN, Primary Examiner

20

U.S. CL. X.R.

96—139 140

25

20

35